# EUROPEAN PATENT SPECIFICATION

(11) **EP 1 783 235 B1**
(45) Date of publication and mention of the grant of the patent: **07.01.2009**
(21) Application number: 05772406.4
(22) Date of filing: 14.07.2005
(51) Int. Cl.: C22C 14/00, C22C 1/02, C22F 1/18

(54) **TITANIUM-BASED ALLOY**
LEGIERUNG AUF TITANBASIS
ALLIAGE A BASE DE TITANE

(30) Priority: 30.07.2004 RU 2004123500
(43) Date of publication of application: 09.05.2007
(73) Proprietor: Public Stock Company "VSMPO-AVISMA Corporation", Sverdlovsk Region 624760 (RU)
(72) Inventor: TETYUKHIN, Vladislav Valentinovich, Moscow, 125284 (RU); LEVIN, Igor Vasilievich, Sverdlovskaya obl., 624760 (RU); TRUBOCHKIN, Alexandr Vladimirovich, Sverdlovskaya obl., 624760 (RU)
(74) Representative: Rupprecht, Kay
(86) International application number: PCT/RU2005/000381
(87) International publication number: WO 2006/014124

(56) References cited:
- EP-A- 0 683 242
- WO-A-03/095690
- WO-A1-03/095690
- DE-A1- 2 719 324
- RU-C1- 2 039 111
- US-A- 5 332 545
- US-A1- 2003 211 003
- US-A1- 2003 223 902

## Description

### Field of the Invention

The invention relates to the field of metallurgy and particularly to the field of development of state-of-the-art titanium alloys used for making high-strength and high-workable articles including large articles, i.e. alloys of high versatility.

Titanium alloys are widely used as aerospace materials, e.g. in airplanes and rockets since the alloys possess tough mechanical properties and are comparatively light.

### Prior state of Art

Known is the most widely used titanium alloy, Ti6A14V alloy (B.A. Kalachyov, I.S. Polkin and V.D. Talalayev. Titanium Alloys of Different Countries. Reference Book. Moscow: VILS, 2000, p. 58-59) - [1]. This alloy was developed in 1950s in the USA. It is characterized by medium strength of 850 up to 1000 MPa and high workability. It is a good material to work by forming: forging, die forging, and extruding. It is widely used in aeronautical and aerospace engineering, shipbuilding, automotive industry, etc., as well as in manufacturing fasteners for various applications. This alloy is good to work by all types of welding including diffusion bonding.

The disadvantage of Ti6A14V alloy is its insufficient versatility. It is difficult to make rolled sheet products, foil, and tubes thereof since the alloy possesses relatively high resistance to deformation, which in case that the deformation temperature becomes below 800°C leads to the generation of defects such as cracks and shortens the life of working tools or necessitates costly tools.

Known is a pseudo-α-titanium alloy Grade 9 (Ti-3Al-2,5V), which is highly capable of cold working (see [1], p. 44, 45). The strength of this alloy is intermediate between that of Ti-6Al-4V alloy and titanium (600-800 MPa). This alloy is used as cold-worked and stress annealed; it is characterized by high corrosion resistance in various media including sea water. This alloy is used in making tubes for hydraulics and fuel systems of airplanes, rockets, and submarines.

The disadvantage of this alloy is also its low versatility since it requires stress relieving in making large structural parts thereof. Therefore, articles have to be annealed which reduces strength of Grade 9 alloy down to 400-500 MPa.

The most close analogue of the invented alloy is α+β-titanium alloy consisting of 3.0-5.0 Al; 2.1-3.7 V; 0.85-3.15 Mo; 0.85-3.15 Fe; 0.06-0.2 O₂, and inevitable impurities (Japanese application No. 3007214 B2, filed Feb. 7, 2000) - prior art.

The disadvantage of this alloy is that it is rich in Fe and Mo and, therefore, is prone to segregation process. In order to reduce possibility of segregational heterogeneity it is required to use a special ingot melting technology, then carry out rolling and forging at a small deformation rate in order to exclude decoration of "beta-flecks", which decreases the productivity.

### Disclosure of the Invention

It is an object of the invention to provide a versatile titanium alloy which requires the least manufacturing costs and is capable of making a wide product mix thereof, such as large forgings and die forgings, as well as rolled sheet products and foil having sufficient strength and plastic properties and structure.

According to the invention an optimum mix of α- and β-stabilizing alloying elements in a semi-finished product is provided.

According to the invention a titanium base alloy is provided consisting of Aluminum, Vanadium, Molybdenum, Iron, and Oxygen in the following ratio, wt.%:

| | |
|---|---|
| Aluminum | 3.5-4.4 |
| Vanadium | 2.0-4.0 |
| Molybdenum | 0.1-0.8 |
| Iron | max 0.4 |
| Oxygen | max 0.25 |
| Ti | balance |

High strength and ductility combined in the invented alloy is achieved through targeted selection and experimental evaluation of the alloying ranges. The content of α- stabilizers (Aluminum, Oxygen) and β-stabilizers (Vanadium, Molybdenum, and Iron) was determined so as to meet a goal objective.

Aluminum is a α-stabilizer for the α +β-titanium alloys, which contributes to the increase of mechanical strength. However in case that Aluminum content is below 3.5%, sufficient strength aimed in this invention cannot be obtained, whereas in case that Aluminum content exceeds 4.4%, the hot deformation resistance is increased and ductility at lower temperatures is deteriorated, which leads to the lowering of productivity.

Vanadium is added to titanium as a β-stabilizer for the α +β-titanitun alloys, which contributes to the increase of mechanical strength without forming brittle intermetallic compounds with titanium. Presence of Vanadium in the alloy impedes formation of α₂-superstructure in α-phase as β-phase stabilizes, and contributes to the increase of both strength and ductility. In case that Vanadium content is below 2%, sufficient strength aimed in this invention cannot be obtained, whereas in case that Vanadium content exceeds 4.0%, the superplastic elongation is decreased by exceedingly lowering of the beta transus. Vanadium content within the range of 2.0-4.0% in this alloy has the merit in which the scrap of the most used Ti6A14V can be utilized.

Molybdenum is added to titanium as a β-stabilizer for the α +β-titanium alloys. In case that Molybdenum is added within the range of 0.1-0.8% this contributes to its full dissolution in α-phase, which enables to obtain the sufficient strength properties without deteriorating plastic properties. In case that Molybdenum content exceeds 0.8% this contributes to the increase of the specific weight of the alloy due to the fact that Molybdenum is a heavy metal and the plastic properties of the alloy are deteriorated. In case that Molybdenum content is below 0.1%, Molybdenum does not contribute to the alloy properties in full.

Iron added to the alloy up to 0.4% contributes to increase of the volume ratio of β-phase decreasing resistance to deformation in hot working of this alloy which leads to evading of the generation of such defects as cracking. In case that Iron content exceeds 0.4%, this generates a segregation phase with beta-flecks in melting and solidifying of the alloy, which leads to heterogeneity of mechanical properties, especially ductility.

Oxygen contributes to the enhancement of mechanical strength by constituting a solid solution mainly in α-phase. In case that Oxygen content exceeds 0.25%, the alloy ductility may be deteriorated.

The alloy may contain up to 0.1% of carbon and up to 0.05% of nitrogen as inevitable impurities; the total quantity of impurities shall not exceed 0.16%.

### Embodiment of the invention

To evaluate the properties of the claimed alloy ingots were melted by the method of double vacuum arc remelt, having the following chemical composition (Table 1).

**Table 1**

| Alloy | Chemical Composition, wt.% | | | | |
|---|---|---|---|---|---|
| | Al | V | Mo | Fe | O |
| 1 | 3.9 | 2.2 | 0.2 | 0.13 | 0.17 |
| 2 | 4.3 | 2.8 | 0.3 | 0.24 | 0.23 |
| 3 | 4.3 | 3.3 | 0.6 | 0.32 | 0.20 |

**Table 2**

| Alloy | | Heat Treatment | Mechanical Properties | | | |
|---|---|---|---|---|---|---|
| | | | σ_{B}, MPa | σ_{0.2}, MPa | δ, % | ψ, % |
| 1 | | W/o annealing | 810 | 735 | 15.2 | 38.2 |
| | | 750°C 1 hour, air | 780 | 693 | 13.2 | 32.0 |
| 2 | | W/o annealing | 960 | 840 | 14.2 | 33.1 |
| | | 750°C 1 hour, air | 920 | 845 | 13.6 | 32.5 |
| 3 | α+β | 710°C 3 hours, air | 900 | 835 | 15 | 33.0 |
| | β | 710°C 3 hours, air | 870 | 800 | 14 | 28.0 |

Bars with the diameter of 50 mm were made of each ingot by hot working. Part of the bars was heat treated by annealing at 750°C, soaking for 1 hour and cooling in the air. The mechanical properties at room temperature were evaluated on the bars heat treated and on those not heat treated. The evaluation results are given in Table 2. In addition, the mechanical properties of β-upset workpieces were evaluated, which were heat treated at 710°C, soaked for 3 hours and cooled in air. The results of mechanical test of workpieces upset in α+β and β-field are given in Table 2.

### Commercial practicability

In comparison with the known alloys the invented alloy is highly versatile, economically beneficial and has lower cost due to the fact that scrap of widely known alloys, such as Ti6Al4V, can be used for its production. This alloy possesses required and sufficient mechanical properties and can be utilized for making a wide range of products, such as large forgings and die forgings, thin sheets and foil, by working in both α+β-field and β-field.

## Claims

1. A titanium base alloy consisting of Aluminum, Vanadium, Molybdenum, Iron, and Oxygen in the following ratio, wt.%:
| | |
|---|---|
| Aluminum | 3.5-4.4 |
| Vanadium | 2.0-4.0 |
| Molybdenum | 0.1-0.8 |
| Iron | max 0.4 |
| Oxygen | max 0.25 |
| Titanium | balance |

## Patentansprüche

1. Titanbasis-Legierung, welche Aluminium, Vanadium, Molybdän, Eisen und Sauerstoff in dem folgenden Gewichtsverhältnis enthält:
| | |
|---|---|
| Aluminium: | 3,5 - 4,4 |
| Vanadium: | 2,0 - 4,0 |
| Molybdän: | 0,1 - 0,8 |
| Eisen: | max 0,4 |
| Sauerstoff: | max 0,25 |
| Titan: | Rest |

## Revendications

1. Alliage à base de titane constitué d'aluminium, de vanadium, de molybdène, de fer et d'oxygène dans les rapports suivants, en pourcentage en poids :
| | |
|---|---|
| aluminium | 3,5 à 4,4 |
| vanadium | 2,0 à 4,0 |
| molybdène | 0,1 à 0,8 |
| fer | maximum 0,4 |
| oxygène | maximum 0,25 |
| titane | le reste. |
